

Patented Aug. 3, 1926.

1,594,770

# UNITED STATES PATENT OFFICE.

ALEX BROOKING DAVIS, OF CINCINNATI, OHIO, ASSIGNOR TO A. B. DICK COMPANY, OF CHICAGO, ILLINOIS, A CORPORATION OF ILLINOIS.

## STENCIL SHEET AND PROCESS OF PRODUCING THE SAME.

No Drawing.

Application filed May 9, 1925. Serial No. 29,234.

This invention is based upon the discovery that a strong, stable and efficient stencil sheet, preferably of the flexible, type-impressible variety, may be produced by the use of metals which may be associated with a suitable fabric such, for example, as the fibrous, porous material known as "yoshino," this association being effected in any one of a variety of ways as hereinafter pointed out. A wide range of metals may be employed, either pure or in the form of alloys, a thin film or films thereof being employed which may be impressed, as by a stylus or the type of a writing machine, to form open characters therein through which ink may be passed for the production of copies upon an underlying impression sheet in the manner practiced in mimeographing.

Within this invention one way of effecting the association of the metal with the fabric sheet is by the reduction of a metallic solution in which the sheet is immersed. Another way is by employing low melting metals or alloys thereof, such as tin, lead, bismuth, cadmium and the like, melting these and rolling a thin film thereof between two fabric sheets on a hot plate or in contact with a single fabric sheet, the fabric sheet or sheets having been, if desired, treated with a suitable strengthening agent, as, for example, an oil-tempered cellulose such as acetone-soluble cellulose acetate or the like.

Another way is to make the fabric sheet (pretreated with a strengthening agent as above described or not) electrically conductive, as by dusting it with carbon or finely divided metals or impregnating it with certain metallic salts and then to deposit the metal thereon (either on one side of the fabric sheet or both) by the process of electrodeposition. Or, if desired, a thin metallic film may be applied to the fabric sheet (which may be pretreated as above described) and permanently attached thereto by a suitable adhesive, as gum damar or sandarac. With stencil sheets prepared in any of the above ways the type or stylus may make contact direct with such sheet, or through a thin type-protecting tissue, and, if desired, a cushion sheet may be employed on which the stencil sheet may rest during the process of stencilization, such cushion sheet being preferably of soft paper or other fabric.

As an example of a suitable method of preparing a metallic stencil under this invention, the following process may be employed. There is prepared a solution of 100 gms. of silver nitrate dissolved in 1000 cc. 60 of water containing 55 gms. of 26 deg. Bé. aqua ammonia. With this solution, there is now mixed another solution consisting of 50 gms. of potassium tartrate dissolved in 1000 cc. of water. This mixture is now diluted with ten times its own volume of water, and there are immersed in the resulting bath sheets of yoshino paper which have been previously strengthened by dipping them through a solution of modified cellulose acetate in acetone and allowing the acetone to evaporate. The silver nitrate is now rapidly reduced to metallic silver by the potassium tartrate, and the silver is deposited in the metallic state as a homogeneous coating upon the yoshino surface. This metallic coating varies in thickness according to the amount of silver deposited or the time that the sheet is immersed and practically any desired thickness of coating 75 may be obtained. When the sheets have thus been coated with silver to the desired extent, they are removed and dried, and then constitute a type impressible stencil sheet capable of yielding large numbers of copies 80 when used on the usual type of duplicating machines.

If only a thin coating of silver be deposited, the sheets may subsequently be immersed in a plating bath of copper or other metals, and an additional coating of metal deposited thereon electrically in known manner.

What I claim is:—

1. A type impressible stencil sheet having a porous base in association with metal. 95
2. A type impressible stencil sheet having a porous base in association with metallic foil.
3. A type impressible stencil sheet having a porous base in association with a metallic alloy. 100
4. A type impressible stencil sheet having a porous base pretreated with a strengthening substance and associated with metal. 105
5. A type impressible stencil sheet having a porous base pretreated with a strengthening substance and associated with metal foil.
6. A type impressible stencil sheet having a porous base pretreated with a strengthen- 110

ing substance and associated with a metallic alloy.

7. In a type impossibly stencil sheet, a sheet of porous material, a metallic film, and means for attaching said sheet and film together.

8. In a type impossibly stencil sheet, a sheet of porous material, a metallic film, and means for attaching said sheet and film together throughout substantially their entire area.

9. The process of preparing a stencil sheet which consists in pretreating a sheet of porous material to strengthen its structure and then permanently associating the same with a metallic film.

10. The process of preparing a stencil sheet which consists in pretreating a sheet of porous material to strengthen its structure and then permanently associating the same

with a metallic film, said sheet and film being in contact throughout substantially their entire area.

11. The process of preparing a stencil sheet which consists in pretreating a sheet of porous material to strengthen its structure and then permanently associating the same with a metallic film on either side thereof.

12. The process of preparing a stencil sheet which consists in applying metal, in finely divided form, to a porous base, constituting thereon a homogeneous film.

13. The process of preparing a stencil sheet which consists in pretreating a porous sheet to strengthen its structure and applying metal, in finely divided form, thereto, such metal constituting a homogeneous film.

This specification signed this 5th day of May, 1925.

ALEX BROOKING DAVIS.